

# UNITED STATES PATENT OFFICE.

OTTOKAR SERPEK, OF MADULEIN, SWITZERLAND.

## METHOD OF PRODUCING ALUMINUM NITRIDS.

No. 888,044.

Specification of Letters Patent. Patented May 12, 1908.

Application filed May 22, 1907. Serial No. 375,452.

*To all whom it may concern:*

Be it known that I, OTTOKAR SERPEK, doctor of chemistry, a subject of the Emperor of Austria-Hungary, residing at Ma-  
5 dulein, Switzerland, have invented new and useful Improvements in Methods of Producing Aluminum Nitrids, of which the following is a specification.

My invention relates to the manufacture  
10 of aluminum nitrids and is carried out in the following manner: A powdered mixture of alumina, carbon and a metal, as for instance, copper or iron, which is capable of forming an alloy with aluminum, is heated in an at-  
15 mosphere containing nitrogen, such as air. Aluminum nitrid is then formed, while at the same time an increase of volume in the volume of the mass takes place.

The temperature to be obtained must be  
20 so high that, if no nitrogen were present, the partial formation of an alloy of aluminum and iron or copper would be initiated. Such a temperature is obtained at red heat, for instance by a coke fire. The temperature in  
25 question is only to be maintained for a short time, because after the formation of the alloy of aluminum and copper or iron has begun, the chemical reaction itself develops a high temperature, so that it is no longer necessary  
30 to heat the mixture by the coke or other fire to such an extent as in the beginning of the process.

The mixture to be treated contains pref-  
erably three parts of alumina and one part  
35 or a little more of carbon, and the metals

mentioned are to be added in a quantity of about 5%.— There may be admixed one single metal or a mixture of two or more metals.

The mass thus produced contains almost 40 pure aluminum nitrids with only an insignificant amount of aluminum carbide, the further treatment of which may be dispensed with. An acid gas such as hydrochloric acid or sulfur dioxide may be advantageously 45 added to the nitrogen, whereby the formation of aluminum nitrids is facilitated. In this case the nitrogen contains about one-tenth of a per cent. of acid gas.

I claim:

1. The method of producing aluminum nitrids which consists in heating a mixture of alumina, carbon and a metal capable of forming an alloy with aluminum in an atmosphere containing nitrogen to red heat, 55 substantially as described.

2. The method of producing aluminum nitrids which consists in heating a mixture of alumina, carbon and a metal capable of forming an alloy with aluminum in an atmosphere 60 containing nitrogen and an acid gas to red heat, substantially as described.

In testimony whereof I have signed my name to this specification in the presence of two subscribing witnesses.

OTTOKAR SERPEK.

Witnesses:

A. LIEBERKNECHT,  
EUGEN TRATE.